

## UNITED STATES PATENT OFFICE

FRITZ EMIL FUCHS, OF EAST ORANGE, NEW JERSEY, ASSIGNOR TO THE SPECIALTY PRODUCTS COMPANY, INC., OF NEW YORK, N. Y., A CORPORATION OF NEW JERSEY

## PAPER MANUFACTURE

No Drawing.

Application filed March 13, 1929. Serial No. 346,814.

The object of this invention, is to produce a transparent paper of some suitable weight and of relatively great strength.

I am aware that tissue papers have been produced, and that tissue papers have been subjected to waxing, and to other treatments which make them transparent to a certain extent. However, the transparency of such papers has been limited by the inability to 10 impregnate the fibres with a material that would give them a transparent appearance, and therefore such papers have been only semi-transparent; that is, they have been streaked, or the fibres thereof, have been 15 plainly evident. An object of my invention, then, is to make a paper almost totally transparent.

The use of papers in wrapping such articles as candy boxes, has been discontinued 20 for the reason that a product has been found wholly transparent and waterproof, the use of which improves the appearance of the package. My object is to make a paper that can be used as a substitute for this other material, which will be equally transparent; 25 equally waterproof, and therefore equally attractive.

Another object of my invention is to produce a transparent paper that may later be 30 waxed, and therefore in obtaining the transparency, I employ a material that will not be wax repellent, and to accomplish these desirable results, I proceed generally as follows:—

35 I produce a good quality of tough paper of desirable weight. A white bond paper is preferred; of course, without the usual water marks. I may use any of the so-called straight grain paper; that is, a "linen" paper, or a straight wood fibre product. This paper is prepared in the ordinary manner, up to the calendering. For the purpose of calendering, water is usually used, but I have 40 found that the addition of soluble, or emulsified, fatty, and mineral oils to the water in

the dampener previous to calendering, will produce a very desirable effect.

In my experiments, I have employed with a high degree of satisfaction, a white emulsified mineral oil, having no odor—being practically non-oxidizing. 50

In my experiments, I have employed approximately a two-percent emulsion, but the percentage must obviously be varied according to the quality, density and construction 55 of the paper, and to the extent of transparency desired, and also the use of different oils will require a difference in the percentage. This treatment allows for subsequent waxing; in fact, a higher degree of lustre 60 is obtainable after this treatment, and I have also found that this treatment results in the production of a paper of greater smoothness and more unity, as the oil serves to soften the fibres and allows the 65 calendering rolls to smooth out the fibres and polish them as well.

I have also found that the use of a small amount of oil will not prevent subsequent gluing, and as a consequence, my paper may 70 readily serve as a wrapper as previously described.

It will of course be understood that the emulsified, or soluble oil is mixed with water, and that dampening and calendering takes 75 place in the usual manner, and therefore what I claim and desire to secure by Letters Patent is:—

1. The production of transparent papers, which consists of dampening the paper prior 80 to calendering, with a solution containing a relatively low percentage of emulsifiable oil in water.

2. The method of producing transparent paper, which consists of dampening the 85 paper prior to calendering, with a relatively low percentage of a non-oxidizing, clear white oil emulsified in water.

3. The method of producing transparent paper, which consists of dampening the 90

paper prior to calendering with a relatively low percentage of non-oxidizing clear white oil, emulsified in water, and later waxing said paper.

5 4. The method of producing transparent paper, of high lustre, which consists of moistening said paper prior to calendering, with an emulsion containing a low percentage of non-oxidizing clear white mineral oil  
10 and water, and thereafter finishing said paper.

FRITZ EMIL FUCHS.

15

20

25

30

35

40

45

50

55

60

65